

## UNITED STATES PATENT OFFICE

2,090,393

## LIQUID FUEL

Arthur A. Roberts, London, England; Arthur Roberts and Clifford Wilbur Smith administrators of said Arthur A. Roberts, deceased

No Drawing. Application July 17, 1934, Serial No. 735,711. Renewed January 11, 1937. In Great Britain June 23, 1933

3 Claims. (Cl. 44—3)

The present invention relates to improvements in liquid or mobile fuels, such as oil or stabilized mixtures of carbonaceous materials, such as coal with oil.

5 It is normally not possible to consume oil or coal-oil mixtures having a water content, as the free water is apt to extinguish the flame.

According to the present invention water is added to a mobile or liquid fuel by emulsification therewith, whereby efficient combustion can be obtained and moreover, it has been found that under certain conditions the intensity of combustion is increased.

10 Various emulsifying agents may be used, such as starch or casein. Either an oil soluble or a water soluble emulsifying agent or both conjointly may be used, such as a sulphonic acid derived from a vegetable oil or a naphthenic acid.

15 Where the fuel is to be used, for instance, in marine work, it will be desirable to use an emulsifier which will operate in the presence of salt or solutions of electrolytes, so that the water content of the fuel will be maintained in emulsification with the fuel in spite of accidental association of the fuel with sea-water or condensed steam.

20 In the application of the invention to coal-oil mixtures or the like the water may conveniently be added as part of the stabilizer for the suspension of the coal particles in the oil where such is employed.

25 Combustion controlling agents, such as boron compounds, may be added and these, if water soluble, may be dissolved in the water addition to the fuel. If desired, non-soluble combustion catalysts, such as one of the oxides of iron may be added to the fuel by suspension therein by means of a stabilizing agent which in coal-oil mixtures may be the same stabilizing agent as used for the coal particles.

30 Intimate emulsification may be obtained by passing the oil with water, or coal dust with oil and water, through a mill, preferably a high speed attrition mill, or a number of such mills in series, which in the case of a coal-oil fuel may also serve to reduce the coal particles to finer size.

35 In the case of a coal-oil fuel the coal may be subjected to grinding with water as a preliminary step prior to treatment for removal of ash forming constituents by any known system, such as for instance, by means of a centrifuge but preferably by a froth flotation process. By this means a substantially ash-free fuel can be obtained which has a high water content, and yet

can be used to form a stable liquid fuel; both solid and water content remain in suspension over any desired storage period.

40 As the addition of water to the oil, or to the coal-oil stabilized mixture by this method will normally tend to increase its viscosity it will, in certain cases, be desirable to reduce the viscosity so that it may be effectively conveyed and consumed. For this purpose materials may be added, such as naphthiaine.

45 By reason of the intimate distribution by means of emulsification of the water throughout the mobile fuel, it will be found that where the fuel is being consumed in a burner this will remain clean, as the dissociation of the water will prevent the partial combustion of the hydrocarbons of the oil or coal and thus prevent the deposit of coke on the burner.

50 It has been found that the efficiency of combustion is remarkably increased by the addition of water to oil or oil-coal stabilized mixtures according to the present invention, as the following comparative tests, taken purely by way of example, will show.

55 A single flue boiler having a rated capacity of 3,000 to 3,500 lbs. of steam per hour and roughly 12 ft. 6 ins. by 6 ft. in size was fired with untreated petroleum oil having a viscosity of 500 seconds on a No. 1 Redwood viscometer.

|                                        |                                        |    |
|----------------------------------------|----------------------------------------|----|
| Specific gravity at 60° Fahrenheit     | 947                                    | 25 |
| Flash point                            | 190° Fahrenheit                        |    |
| Viscosity at 100° Fahrenheit           |                                        |    |
| heft                                   | 480                                    | 35 |
| Ash                                    | 0.08%                                  |    |
| Hard asphalt                           | 3.3%                                   |    |
| Water                                  | 0.15%                                  |    |
| Coke (Conradson)                       | 8.7%                                   |    |
| Sediment                               | 0.22%                                  |    |
| Sulphur                                | 1.07%                                  |    |
| Cold test                              | 10° Fahrenheit                         |    |
| Calorific value                        | 18,900 British thermal units per pound |    |
| Duration of test 9 P. M.<br>to 4 A. M. | 7 hours                                | 45 |
| Quantity of water evaporated           | 4660-3566 gallons                      |    |
| Temperature of feed water              | 51° Fahrenheit                         | 50 |
| Weight of water used                   | 10940 pounds weight                    |    |
| Pounds of steam generated              | 1563 pounds weight                     |    |
| Quantity of oil consumed               | 86.0-42 inches                         | 55 |

|                                                                                                                                                                                      |                                    |
|--------------------------------------------------------------------------------------------------------------------------------------------------------------------------------------|------------------------------------|
| Capacity of tank                                                                                                                                                                     | 1"-2547 gallons                    |
| Average temperature of oil                                                                                                                                                           | 180° Fahrenheit                    |
| Specific gravity of oil                                                                                                                                                              | 0.947                              |
| 5 Specific gravity of oil at 180° Fahrenheit                                                                                                                                         | 0.899                              |
| Weight of oil used                                                                                                                                                                   | 1008 pounds weight                 |
| Calorific value of oil                                                                                                                                                               | 18,900 per pound weight            |
| 10 Weight of water evaporated per pound oil                                                                                                                                          | 10.86 pounds                       |
| Evaporation from and at 212° Fahrenheit                                                                                                                                              | 13.03 pounds                       |
| Steam pressure of boiler                                                                                                                                                             | 100 lbs./sq. in gauge              |
| 15 Total heat used per lb. steam                                                                                                                                                     | 1189 British thermal units         |
| Corrected figure with feed water at 31°                                                                                                                                              |                                    |
| 20 Fahrenheit                                                                                                                                                                        | 1170 British thermal units         |
| British thermal units used in generating                                                                                                                                             |                                    |
| 10.86 pounds weight                                                                                                                                                                  |                                    |
| 25 steam                                                                                                                                                                             | 12076.2                            |
| Actual efficiency at 51° Fahrenheit                                                                                                                                                  | 12076.2/18900=67.2%                |
| 30 The CO <sub>2</sub> content of the flue gases was practically constant throughout the run and varied from 11% to 12% except for the few minutes occupied in changing the burners. |                                    |
| The average mean temperature throughout the test was 1280° centigrade.                                                                                                               |                                    |
| 35 An oil emulsified with 4% of water using one-eighth of 1% of starch as emulsifier was then consumed under identical conditions with the following result:—                        |                                    |
| 40 Duration of test                                                                                                                                                                  | 6 hours (10.30 P. M.—6.30 P. M.)   |
| Quantity of water evaporated                                                                                                                                                         | 12825-11255 gallons                |
| Temperature of feed water                                                                                                                                                            | 57° Fahrenheit                     |
| 45 Weight of water used                                                                                                                                                              | 15700 pounds                       |
| Weight of steam generated/hour                                                                                                                                                       | 1962 pounds                        |
| Quantity of oil consumed                                                                                                                                                             | 80-17,375"                         |
| 50 Capacity of tank                                                                                                                                                                  | 1"-2.5478 gallons                  |
| Average temperature of oil                                                                                                                                                           | 140° Fahrenheit                    |
| Specific gravity of oil                                                                                                                                                              | .907 at 161° Fahrenheit            |
| Specific gravity of oil                                                                                                                                                              | 907 at 161° Fahrenheit             |
| 55 Weight of oil used                                                                                                                                                                | 1440.5 pounds                      |
| Weight of water evaporated per pound of oil                                                                                                                                          | 10.9 pounds                        |
| Steam gauge pressure                                                                                                                                                                 | 94 pounds per square inch          |
| 60 Evaporation from/and at 212° Fahrenheit                                                                                                                                           | 13.00                              |
| Calorific value of fuel                                                                                                                                                              | 16,710 British thermal units/pound |
| Total heat used per pound steam                                                                                                                                                      | 1188 British thermal units         |
| 65 Corrected with feed water at 64° Fahrenheit                                                                                                                                       | 1163 British thermal units         |
| British thermal units used in evaporating                                                                                                                                            |                                    |
| 10.9 lbs. water                                                                                                                                                                      | 12,676                             |
| Actual efficiency                                                                                                                                                                    | 67.7%                              |
| 70 75 CO <sub>2</sub> in flue gases                                                                                                                                                  | 10%                                |

The average mean temperature was found throughout this test to be 1300° centigrade. Moreover, it was found that, while with the untreated or dry oil it was necessary to clean the burners every four hours owing to the considerable quantity of coke deposit forming beneath the flame, with the burners using the treated oil, that is to say, the oil containing the water, only about half the amount of coke deposit had accumulated on the burners after six hours, as compared with the previous accumulation in four hours.

A third test under identical conditions was effected with the same basic medium; that is to say, Anglo-American Petroleum oil having a viscosity of 500 seconds on No. 1 Redwood viscometer, four parts of water being added emulsified by means of one eighth of one part of starch together with three eighths of one part of borax or boric acid in solution in the water and three eighths of one part of sodium chloride in solution in the water, per hundred parts by weight of oil.

It may here be stated that sodium chloride whilst normally acting as a combustion retarding agent is believed to have a retarding effect solely upon the rate of combustion, whilst the boron compound addition has a remarkable effect in increasing the intensity of combustion. This test has had as a result:—

|                                                                          |                            |
|--------------------------------------------------------------------------|----------------------------|
| Duration of test                                                         | 4 hours 3 p. m. to 7 p. m. |
| Quantity of water evaporated                                             | 18703-17908 gallons        |
| Temperature of feed water                                                | 60° Fahrenheit             |
| Weight of water used                                                     | 7950 pounds                |
| Weight of steam generated/hour                                           | 19875 pounds               |
| Quantity of oil consumed                                                 | 29.36"                     |
| Capacity of oil tank                                                     | 1"-2.5478 gallons          |
| Average temperature of oil                                               | 140° Fahrenheit            |
| Weight of oil used (Sp. Gr.-912 at 140° Fahrenheit)                      | 683.5 pounds               |
| Weight of water evaporated per pound oil                                 | 11.63 pounds               |
| Steam gauge pressure                                                     | 90 pounds                  |
| Evaporation from and at 212° Fahrenheit                                  | 13.89                      |
| Calorific value of dry fuel                                              | 18,900                     |
| Calorific value of dry fuel plus 4% water                                | 18,144                     |
| Total heat used per pound steam British thermal units used in converting | 11.63                      |
| pounds water                                                             | 13,491                     |
| Actual efficiency                                                        | 74.35%                     |

The average mean temperature was 1320° centigrade.

It can readily be ascertained that similar tests with stabilized coal-oil mixtures having a water content and stabilized coal-oil mixtures having a water content together with combustion promoting agents would give similar results in increase in efficiency.

Satisfactory combustion has been obtained with oil and oil-coal stabilized mixtures with the water content as high as 10%, although in such cases the combustion efficiency would not be as high as with a lower water content. It will however, be

appreciated that a considerably cheaper fuel can be obtained by this means giving equivalent efficiency to an untreated oil with the additional advantages of burner cleanliness in operation.

5 Fuels manufactured according to the present invention will also be suitable for use in internal combustion engines, for instance, of the self-ignition type.

I declare that what I claim is:—

10 1. A liquid fuel comprising an emulsion of fuel oil with water, said water component having dissolved therein a compound of the group consisting of boric acid and water-soluble borates for controlling the combustion and said water component also having therein an emulsifying and stabilizing agent of the group consisting of starch and casein and characterized by being operative in the presence of electrolytes.

15 2. A liquid fuel comprising an emulsion of fuel

oil with water, said water component having dissolved therein boric acid for controlling the combustion and an emulsifying and stabilizing agent of the group consisting of starch and casein and characterized by being operative in the presence 5 of electrolytes.

3. A liquid fuel comprising an emulsion of fuel oil with substantially 4% of water, said water component having dissolved therein a water-soluble boron-oxygen compound for controlling 10 the combustion and an emulsifying agent of the group consisting of starch and casein and characterized by being operative in the presence of electrolytes, the total quantity of boron-oxygen compound and emulsifying agent being substantially one-half of 1% by weight of the emulsion, and particles of powdered coal suspended in the emulsion. 15

ARTHUR A. ROBERTS.